

# UNITED STATES PATENT OFFICE.

AUGUSTE J. ROSSI, OF NIAGARA FALLS, NEW YORK, ASSIGNOR TO THE TITANIUM ALLOY MANUFACTURING COMPANY, OF NEW YORK, N. Y., A CORPORATION OF MAINE.

## METHOD OF TREATING FERRO METALS.

1,003,805.

Specification of Letters Patent. Patented Sept. 19, 1911.

No Drawing.

Application filed November 20, 1908. Serial No. 463,610.

To all whom it may concern:

Be it known that I, AUGUSTE J. ROSSI, a citizen of the United States, and a resident of Niagara Falls, in the county of Niagara and State of New York, have invented certain new and useful Improvements in Methods of Treating Ferro Metals, of which the following is a specification.

Such metals, as is well known, when melting, absorb gases, being for instance oxidized, to an extent, during fusion, the resulting oxids dissolving in the metal with the result that said metals cannot, in many instances, be cast without developing "blow holes" and other imperfections in the resulting product; other gases, such as nitrogen, are also during the fusion undesirably developed in the molten mass with characteristic malign effects, so that it may be said that hitherto such metals have too frequently contained, or absorbed in melting, noxious elements, or compounds, injuriously affecting the final product. I have discovered that if to such metals when charged into the crucible, or while melting, or molten, there be added a small quantity, preferably from 1% to 2% in weight, of an alloy of a ferro-metal as for instance iron, or steel, and titanium containing say from 5% to 12% of titanium or thereabout, such undesired elements and compounds will be, thereby, largely eliminated from the resulting ferro product, and exceptional hardness and tensile strength, besides other advantages, imparted thereto.

For example my present invention may be practiced as follows:—The ferro-metal to be treated, for instance iron or steel, is melted as usual in the crucible or other container. There is then added thereto an alloy of iron and titanium such as described and claimed in U. S. Letters Patent No. 609,466 or No. 721,467, granted to me respectively on August 23rd 1898 and February 24th 1903, which addition in many cases need not exceed from 1% to 2% of the entire weight of the ferro-metal treated thereto, and the content of titanium 5% to 12% of the said addition, the function of the titanium when added in these comparatively minute proportions being limited to the elimination of the aforesaid undesired compounds or elements, such as oxygen, nitrogen and their compounds and the prevention of the development, or formation, there-

of in the ferro mass while in molten state, the said additions of titanium being, in such cases, so proportioned as to enable my said novel process to result in a final product comparatively free from the said undesired compounds, or elements, or undesired resultants thereof, and containing also not to exceed traces of titanium, say a fraction of 1% at the most. If steel is treated by my said process it will be understood that an alloy of steel and titanium such for instance as results from the process of Letters Patent No. 822,305 granted to me June 5, 1906 may be employed instead of the said alloy of iron and titanium, though I have found the latter preferable.

For the better understanding of my said process of treatment and its results, as compared to the prior art, the following actual operations may be noted, viz:—

1. In a usual steel crucible furnace was charged and melted 100 lbs. of steel, or the proper materials to make it, which, when at the proper temperature were cast in an ingot mold according to the usual practice in such cases. The resulting ingot, weighing 100 lbs., was broken and found to contain blowholes and to show signs of segregation.

2. Then, according to said novel process, was charged another lot of 100 lbs. steel, or of materials proper to make it, into a similar crucible, with the addition of 1 to 2 per cent. in weight of the above mentioned alloy of iron and titanium now known in the trade as a "ferro-titanium," containing 10 to 12 per cent. titanium or thereabout. The conditions and procedure in this case were, in all respects, similar to those in the above described previous instance. The metal was submitted to the same heat until the addition was incorporated. It was then cast in the same kind of molds as were used in the previous instance. The resulting ingot was found to be perfectly solid and, when broken, showed a close grained, dense structure, without blowholes or cavities. Comparative physical tests were made of test bars, made respectively from the metal non-treated and the metal treated, according to the above description. The bars made of the metal treated by said novel process were found to have an ultimate strength, elongation and elastic limit considerably above those of the

bars made of the metal not treated by said process. Scarcely a trace of titanium, when any, was found, by analysis, in the bars treated, thus demonstrating that the action of the titanium ingredient was substantially 5 confined to the elimination, or prevention, of obnoxious gases or oxids, such as oxygen and nitrogen, and the reduction of the oxid of iron formed during the melting of the metal. Similar operations were repeated 10 with additions of  $\frac{1}{2}$  and even  $\frac{1}{4}$  of 1 per cent. and occasionally less of ferro-titanium with equally satisfactory results, the amount of the ingredient added depending on the 15 more or less state of purity of the original steel treated and the greater or lesser amount of obnoxious gases this said steel might contain. Analyses of different parts of the ingot treated showed that there was no practical segregation at certain points, of the 20 different elements of which steel is composed, such as carbon, phosphorus, silicon, contrarily to what is observed in the non-treated metal.

3. Operations of the same nature were repeated with converter steel, the additions of ferro-titanium being made as the metal was poured from the converter into the receiving ladle before casting the molten steel 30 from said ladle in the large ingot molds, as is practiced in converter steel works. The ingots of treated metal were found to be perfectly solid, showing a close grained, dense structure, without blow-holes and 35 showing no segregation, or slag interposed between the layers of metal. Comparative test bars made from the original steel non-treated and from the same after additions of ferro-titanium showed, as before described, 40 in the physical tests, the same increased ultimate strength, elongation and elastic limit above those of the non-treated metal. Scarcely a trace of titanium, when any, was found by analysis in the bars treated, thus 45 demonstrating that the action of the titanium ingredient was substantially confined, as before, to the elimination of obnoxious gases, such as oxygen and nitrogen, and reduction of the oxid of iron formed in the 50 metal, in other words to one of purification. Analyses showed that the oxid of iron, found present in the metal non-treated, to the extent of 0.25 per cent. to 0.30 per cent., had been completely eliminated,—analyses of 55 the treated steel showing “oxid of iron *nil*”, and that the original nitrogen had been reduced to 0.004 per cent., and even to practically nothing, according to the percentage of alloy added. Microscopic examinations 60 showed also the complete absence of the “slag” visible in the ingot non-treated.

4. Operations of the same nature were repeated in the open hearth, following the *modus operandi* used for this kind of steel, 65 the treated metal showing the same supe-

riority in the physical tests and the same purity and freedom from obnoxious elements, gaseous or otherwise, as compared to the original metal, scarcely a trace of titanium, when any, being found in the 70 metal treated.

5. Results entirely comparable were also obtained with cast iron treated, either in the ladle or cupola, with additions of ferro-titanium. The metal treated showing, in all 75 cases, a greater resistance in the physical tests, a close grained dense structure; and the absence of blow-holes, oxids or slags, being again a prominent feature, though but a trace, if any, of titanium was found in 80 the treated metal.

The effects of my said process are also advantageous in cases in which the molten ferro-metals are intended to form the basis of alloys of such metals with others, as for instance nickel, chromium, tungsten, molybdenum, etc. the resulting alloys derived from the ferro-metals so treated by my said process containing also not to exceed 1% or traces of titanium and being comparatively 90 free from blow-holes, and in many other respects superior to those produced without the aid of my process. In the production of such alloys the titanic purifier may be either introduced into the molten mass composed of all the constituent metals, or preliminarily, as aforesaid, into the ferro-metal, afterward assembled with another not so treated, to produce the desired alloy.

It will be observed that in practicing my 100 present invention it is always preferable to regulate the titanium introduced to an amount merely sufficient to take up, as fully as possible, in chemical combination with itself, the undesired elements and compounds 105 contained, or developed in, the particular ferro-metal under treatment, as these may be determined by test and experience in each case.

I am aware that titanium has heretofore 110 been employed with ferro-metals as described in my said patents, but only with intent and effect of producing, as final product, an alloy containing a required percentage of titanium, which alloy might in turn, 115 if desired, be employed for so-called “seasoning” of iron or steel, *i. e.* incorporating into the latter a lower but likewise predetermined positive content of titanium, with expectation of thereby imparting to the final 120 product desirable characteristics of that metal *per se*.

I am also aware that titanic acid, *i. e.* the chemical compound of titanium with oxygen, has been introduced, in relatively small 125 percentages, into molten cast iron, the said titanic acid being, in this instance, preliminarily mixed with a metal capable of reacting therewith, as for instance aluminium, and that the expectation has been hazarded 130

that, in such case, the titanium has either been taken up by the molten cast iron or absorbed by gases contained in latter, the result being homogeneous casting. Aside 5 from the irrationality of such expectation, due to the introduction of the titanic element in a form in which its affinities are already satisfied, *i. e.* in the form of an oxid, the extreme refractoriness of which is 10 well known, I do not wish to be understood as claiming such procedure as any part of my present invention.

I am also aware that pig-iron produced from titaniferous ores in the blast furnace 15 has been asserted to contain sometimes a fractional percentage of titanium, the presence of which however has been due to indirect causes, irregular, unreliable, dependent upon special or accidental conditions, 20 such as are uncontrollable by the founder, and which may often interfere with the proper and regular running of the furnace. I do not wish to be understood as claiming herein any such procedures or resulting 25 products, my present inventions being distinguishable therefrom in that the latter involve, as I believe for the first time, the discovery that titanium *per se* in metallic state operates in exceptional degree as an absorb- 30 ent, or eliminator, of undesirable elements and compounds from molten ferro-metals, and the designed introduction into the presence of such metals, while molten, of merely sufficient metallic titanium to absorb, or 35 eliminate such undesired compounds and elements, and without leaving in the final product to exceed traces of said titanium, from which procedure results articles possessing novel and desirable characteristics, 40 it being for some purposes desirable that titanium, owing to its affinities and for other reasons, should be substantially eliminated from ferro-metal products.

I am also aware that it has been hereto- 45 fore suggested that alloys of titanium with other than ferro-metals, as for instance alloys of titanium and aluminium, alloys of titanium and calcium, also alloys of iron with titanium in combination with metallic 50 borids, might be advantageously employed to improve the quality of iron and steel, and I do not therefore wish to be understood as

claiming any such procedures, which differ from mine in their dependence upon agents other than titanium to accomplish the de- 55 sired result, or, and also, in providing for retention of a substantial content of titanium in the final product and dependence upon such content.

It is also to be noted that the introduction, 60 into the bath, of titanium alloyed with the ferro-metal treated, or as ferro-titanium, as well as such introduction per said alloys comparatively low in titanium content, im- 65 portantly facilitates and increases uniform dissemination and superior desired action of the titanium throughout the bath.

Having thus described my invention, what I claim as new and desire to secure by Letters Patent is the following, viz:— 70

1. The method of treating a ferro-metal which comprises incorporating therewith while molten a quantity of the alloy of a ferro-metal with metallic titanium, the said titanium being proportioned to combine 75 with undesired compounds and elements and secure a final product containing substantially no titanium.

2. The method of treating steel which comprises incorporating therewith while 80 molten a quantity of the alloy of iron with metallic titanium, the said titanium being proportioned to combine with undesired com- 85 pounds and elements and secure a final product containing substantially no titanium. 85

3. The method of treating iron which comprises incorporating therewith, while molten, a quantity of the alloy of iron with metallic titanium, the said titanium being proportioned to combine with undesired com- 90 pounds and elements and secure a final product containing substantially no titanium. 90

4. The method of treating ferro-metals which comprises incorporating therewith while molten a quantity of a ferro-metal as- 95 sociated with metallic titanium, the said titanium being proportioned to combine with undesired compounds and elements and secure a final product containing substan- tially no titanium. 95

AUGUSTE J. ROSSI.

Witnesses:

ED. A. BRUCKNER,  
WILLIAM F. MEREDITH.